

April 12, 1938.

N. L. HARRIS ET AL

2,113,984

QUARTZ SEAL

Filed Sept. 28, 1937



Inventors:  
Norman L. Harris,  
John W. Ryde,  
by *Harry E. Dunham*  
Their Attorney.

## UNITED STATES PATENT OFFICE

2,113,984

## QUARTZ SEAL

Norman L. Harris and John W. Ryde, Middlesex,  
England, assignors to General Electric Com-  
pany, a corporation of New York

Application September 28, 1937, Serial No. 166,226  
In Great Britain June 30, 1936

5 Claims. (Cl. 176—126)

Our invention relates to the sealing of metal to vitreous material and more particularly to hermetically sealing electric conductors into or through quartz wherein the conductor, preferably in the form of a very thin strip, may be placed within a quartz tube which is then caused to collapse onto the strip by externally applied heat. When the metal of the conductor is tungsten or molybdenum, the thickness of the strip should not exceed 20 microns, a thickness of 10 to 15 microns being usually preferable. This process is particularly valuable in the manufacture of high-pressure metal-vapour lamps with quartz envelopes, such as those disclosed in United States application Serial No. 46,952, Bol et al., filed October 26, 1935, Patent No. 2,094,694.

It is known that if the metal is oxidizable, like tungsten or molybdenum, the space between the strip and the quartz tube must be evacuated, or otherwise rendered free from oxidizing gases, before the quartz is heated for the formation of even a thin film of oxide on the metal makes it impossible to obtain a satisfactory seal. The manufacture of the seal is thereby complicated. The object of this invention is to provide a modification of the said process in which, although an oxidizable refractory metal is used, the seal can be made without removing oxidizing gases.

According to the invention, this object is attained by coating the strip, before it is heated within the quartz tube, with a layer of a refractory non-oxidizable metal, which is preferably rhodium, the said layer being much thinner than the strip. "Refractory" means having a melting point substantially higher than the softening temperature of quartz. Since it is essential that the strip should be very thin, the thickness of the coating must be sufficient to prevent oxidation, and yet not so great as to interfere with the process of sealing.

The drawing is a longitudinal sectional view, on an enlarged scale and taken at an angle to show the strip in perspective, of a high pressure lamp of the type disclosed in the above-mentioned Patent 2,094,694.

Referring to the drawing, the lamp comprises a tubular quartz envelope 10 containing thermionic electrodes 11—11 each of which is supported by a lead-in conductor comprising wires 12 and 13, of tungsten for example, welded to the ends of the strip 14 which is sealed directly into the end portion of the envelope 10. The strip 14, in accordance with our invention, consists preferably of molybdenum or tungsten having a coating of rhodium thereon.

The preferred method of forming the layer or coating is by the known process of distillation. For this purpose the uncoated clean strip may be placed in a vacuum adjacent to a tungsten helix enclosing a bead of rhodium, and the tungsten

heated by a current passed through it until the rhodium evaporates and is deposited on the strip. Since the strip has to be coated on all sides, the process may be repeated with different surfaces of the strip turned towards the helix, or it may be surrounded by several helices each containing a rhodium bead. Several strips may be coated at the same time.

Alternatively, the thin layer may be formed by the known process of cathodic sputtering or even by electro-plating.

The layer need not be more than 1 micron thick. Thus with a molybdenum strip 10 microns thick and a few millimeters wide, a layer of rhodium 0.75 micron thick has been found satisfactory.

In the sealing of the strip 14 to the quartz tube 10, although complete removal of the air is not necessary, partial removal is desirable in order that the collapse of the tube onto the strip may be aided by the external pressure, a reduction of the pressure of the air within the tube by about one-quarter being sufficient. Alternatively the pressure may not be reduced at all, and collapse aided by mechanically applied pressure, as in the known process of making a pressed seal.

What we claim as new and desire to secure by Letters Patent of the United States is:

1. In combination with an article of quartz, a conductive member sealed directly therein and consisting of an oxidizable refractory metal not substantially greater than twenty microns thick and having thereon a coating of rhodium of a thickness much less than that of said conductive member.

2. In combination with an article of quartz, a conductive member sealed directly therein and consisting of an oxidizable refractory metal not substantially greater than twenty microns thick and having thereon a coating of rhodium of a thickness of less than one micron.

3. In combination with an article of quartz, a conductive member sealed directly therein and consisting of a strip of molybdenum not substantially greater than twenty microns thick and having thereon a coating of rhodium of a thickness of less than one micron.

4. In combination with an article of quartz, a conductive member sealed directly therein and consisting of an oxidizable refractory metal having thereon a very thin coating of rhodium.

5. In combination with an article of quartz, a conductive member sealed directly therein and consisting of a strip of tungsten not substantially greater than twenty microns thick and having thereon a coating of rhodium of a thickness of less than one micron.

NORMAN L. HARRIS.  
JOHN W. RYDE.